

April 13, 1937.

G. I. THURMOND

2,076,801

PROCESS FOR PRODUCING ARTIFICIAL SILK

Filed Nov. 24, 1933



Fig. 1.



Fig. 2.



Fig. 3.



Fig. 4.

INVENTOR  
Gilbert I. Thurmond  
BY Albin F. Knight  
ATTORNEY.

## UNITED STATES PATENT OFFICE

2,076,801

## PROCESS FOR PRODUCING ARTIFICIAL SILK

Gilbert I. Thurmond, Asheville, N. C., assignor to  
American Enka Corporation, Enka, N. C., a corporation of Delaware

Application November 24, 1933, Serial No. 699,629

12 Claims. (Cl. 18—54)

This invention relates to artificial silk filaments and to the manufacture of the same, and more particularly to the product and the production of viscose threads and the like by the so-called 5 stretch spinning process.

The process broadly includes means for extruding the viscose solution through very fine openings into a coagulating bath from which it is carried off by suitable thread guides or rollers 10 to the bobbin or pot, as the case may be. During its path of travel the thread is subjected to a stretching action.

Past practices involving the stretch-spinning method in the production of artificial silk filaments have resulted in the encounter of numerous difficulties, one of which, being that after the thread has been wound on the bobbin and treated in the ordinary manner and subsequently dyed, the rate of dyeing or the rate of the absorption 20 of the dye is higher on the outside layers of the yarn. Earlier results were also disadvantageous in that a difference in the color intensity of the dyed yarn occurred throughout the yarn package.

25 The reason for the above referred to differences in the dyeing of the thread is due to the fact that the inner layers of thread are wound on a substantially rigid form and cannot therefore contract to an appreciable extent, while the outer 30 layers are able to contract to a larger degree.

It is an object of the present invention to overcome the difficulties heretofore encountered by the production of yarn having varying dye absorption properties, and to produce artificial silk 35 threads by the stretch-spinning process which will have substantially uniform dyeing characteristics.

A further object of this invention is to provide a process for stretching the yarn in a constantly increasing manner from the inside to the outside 40 of the bobbin upon which it is wound.

It is further contemplated to employ a suitable apparatus in which this process can be carried out.

Other objects will appear from the following 45 description when considered in connection with the accompanying drawing wherein,

Fig. I is a diagrammatic side view of one form of the apparatus for practicing the present method.

50 Fig. II is a top view of the mechanism shown in Fig. I.

Fig. III is a diagrammatic side view of a modified form of the apparatus for practicing this 55 invention, and

Fig. IV is a top view of the modified form of the apparatus shown in Fig. III.

Referring to Figures I and II, 1 designates the spinnerette from which the yarn 2 is extruded. The yarn 2 is led around the godet wheel 3 one 5 or more times and thence carried to a second godet wheel 4. After the yarn has been wound around the second godet wheel 4 one or more times it may, if desired, be led around a roller 5. Finally the yarn is wound upon a bobbin 6. 10

The godet wheels 3 and 4 are positively driven by any suitable means (not shown). The peripheral speeds of these two wheels are maintained different so that a constant stretching action is given to the yarn between the two wheels. During 15 the period of winding the yarn on the bobbin, the peripheral speeds of the two godet wheels are maintained constantly different but at the same time the peripheral speeds of the two godet wheels are gradually decreased. This decrease in speed 20 is predetermined and may be carried out by any suitable driving means such as cone pulleys.

The bobbin 6 runs at a lower peripheral speed 25 at all times than the peripheral speed of the godet 4 whereby a reduced tension is effected on the yarn between the bobbin and the godet wheel, thereby allowing a certain amount of contraction in the yarn at this stage.

The rotary speed of the bobbin is gradually decreased to compensate for the increase in diameter of the yarn as it builds up on the bobbin. This results in a constant peripheral speed of 30 the bobbin.

Owing to the decrease in the peripheral speed 35 of the godet wheel 4 and the constant peripheral speed of the bobbin 6, the tension between the godet wheel and the bobbin is gradually increased as the diameter on the bobbin increases thereby maintaining less contraction of the yarn progressively from the inside to the outside. 40

The process, therefore, in its final analysis provides for a constant stretching of the yarn and a constant decrease in contraction of the yarn. The result of processing the yarn in such a manner is that as the yarn is wound on the bobbin 45 it has an ever increasing elongation, so that when the yarn has been dried on the bobbin, owing to the contraction, an equal tension exists throughout the yarn package which will, therefore, permit uniform dyeing throughout, as the 50 dye rate decreases in direct proportion to the increase of elongation of the filaments.

Whereas the godet wheels 3 and 4 have been described as having different peripheral speeds and constantly decreasing rates of speed, there- 55

by producing a substantially constant stretch, they may where desirable have different peripheral speeds and different decreasing rates in speed, wherein a variable stretch will take place 5 between these points, or one of the wheels may be maintained at a constant speed thereby also effecting a variable stretch. If a variable stretch is effected then a substantially constant contraction is desired and this can be obtained by estab- 10 lishing approximately the same peripheral speed between the godet wheel 4 and the bobbin 6. The results obtained by the practicing of either of the processes referred to are generally the same; that is a yarn is formed with increased 15 elongation from the inside to the outside of the bobbin.

In the modification shown in Figures 3 and 4, a thread guide 7 may be substituted for the first godet wheel 3. In the use of this modified form 20 of apparatus the stretching action takes place between the thread guide 7 and the godet wheel 8. The speed of the godet wheel 8 is gradually decreased during the operation. At the same time the bobbin 9 is operated with a substan- 25 tially constant peripheral speed. However, under practical conditions it is customary to increase the peripheral speed of the bobbin slightly during the formation of a complete package. Now, between the peripheral speed of the godet 30 wheel 8 and the bobbin 9 several relations may exist; for instance, the peripheral speed of the bobbin may be less than the speed of the godet wheel during the complete formation of the yarn package, or the peripheral speed of the bobbin 35 may be less during the beginning of the package formation and, due to the above mentioned increase of this speed, may at the end of the package formation become even slightly greater than the speed of the godet wheel. In the first 40 case as mentioned above, during the formation of the package the rate of contraction is gradually decreasing. In the second case, during the beginning of the spinning the stretch is de- 45 creasing and is towards the end of the formation of the package gradually replaced by a certain elongation given to the freshly spun yarn package.

Whereas the apparatus and process has been described as applied to the drawing, various 50 other modifications and changes may be made to fall within the scope of the invention.

Having thus described my invention, what I claim is:

1. The process of producing artificial silk 55 thread and the like of substantially uniform denier and having improved dyeing properties by gradually increasing the elongation of the thread as it is formed into a package which comprises the steps of extruding a cellulosic 60 solution to form a thread, conducting the thread as formed to a bobbin and giving the thread different linear speeds at pre-determined spaced points in its path of travel while directly propelling the same at one or more points in advance 65 of the bobbin to effect a stretching of the thread, and changing the difference in the linear speeds of the thread at the said spaced points by gradually changing the speed of propulsion at the one or more propulsion points, whereby objectionable characteristics resulting from contraction 70 are avoided.

2. The process of producing artificial silk 75 thread and the like of substantially uniform denier, and having improved dyeing properties by gradually increasing the elongation of the

thread which comprises extruding a cellulosic solution to form a thread, giving the thread different linear speeds at pre-determined spaced points in its path of travel by directly propelling the same in advance of a bobbin so as to stretch the thread, and during the formation of a complete package, changing the difference in the linear speeds of the thread at the said spaced points by gradually decreasing the speed of propulsion at the one or more propulsion points in 10 advance of the bobbin, whereby objectionable characteristics resulting from contraction are avoided. 5

3. The process of producing artificial silk 15 thread and the like of substantially uniform denier and having improved dyeing properties which comprises extruding a cellulosic solution to form a thread, giving the thread different linear speeds at pre-determined spaced points in its path of travel by directly propelling the same in advance of a bobbin so as to stretch the thread, gradually increasing the difference in the linear speeds of the thread at the said spaced points by changing the speed at the point of 20 propulsion, winding the thread upon the bobbin at a reduced tension thereby permitting contraction of the thread beyond the spaced points, and reducing the amount of contraction during the winding of the thread upon the bobbin by gradually increasing the winding tension, whereby 25 objectionable characteristics resulting from contraction are avoided. 30

4. The process of producing artificial silk 35 thread and the like of substantially uniform denier and having improved dyeing properties which comprises extruding a cellulosic solution to form a thread, giving the thread different linear speeds at pre-determined spaced points in its path of travel by passing the same around a godet at several spaced points in advance of a 40 bobbin so that the linear speeds of the thread at the spaced points are substantially equal to the peripheral speeds of the respective godets which directly propel the same so as to stretch the thread, gradually reducing the linear speed 45 of successive portions of the thread as it passes between the spaced points by reducing the peripheral speeds of the godets while constantly stretching the succeeding portions of the thread, and forming a package by winding the thread onto the bobbin while the thread is maintained under a tension which varies in accordance with the tension on the thread between the said spaced 50 points in such manner as to give a gradual elongation of the thread as the package is being formed therefrom whereby objectionable characteristics resulting from contraction in the package are avoided. 55

5. The process of producing artificial silk 60 thread and the like of substantially uniform denier and having improved dyeing properties which comprises extruding a cellulosic solution to form a thread, giving the thread different linear speeds at pre-determined spaced points in its path of travel in advance of a bobbin by passing 65 the same around a godet at each of the spaced points so that the linear speeds of the thread at the spaced points is substantially equal to the peripheral speeds of the respective godets and which directly propel the same so as to stretch the thread, gradually decreasing the rate of withdrawal of the thread as it is formed by decreasing the peripheral speed of the godet at the pre-determined point first passed by the thread and operating the godet at the other pre-determined 70 75

point at such peripheral speed as to subject succeeding portions of the thread to substantially constantly changing stretch, and winding the thread thus stretched upon a bobbin rotating at a constant peripheral speed to maintain the thread as wound under a constant tension, whereby objectionable characteristics resulting from contraction are avoided.

6. In the manufacture of artificial silk, a process for preparing threads, filaments and the like which comprises spinning a cellulosic solution to form a thread, drawing the thread from a coagulating medium by a driven godet, passing the thread to a point of collection under substantially no tension during the initial spinning operation and thereafter increasing the tension as the spinning operation continues.

7. In the manufacture of artificial silk, a process for preparing threads, filaments and the like which comprises spinning a cellulosic solution to form a thread, drawing the thread from a coagulating medium by a driven godet, passing the thread to a point of collection under substantially no tension during the initial spinning operation and thereafter increasing the tension between the godet and point of collection as the spinning operation continues.

8. In the manufacture of artificial silk, a process for preparing threads, filaments and the like which comprises spinning a cellulosic solution to form a thread, drawing the thread from a coagulating medium by a driven godet, passing the thread to a bobbin rotating at a lower peripheral speed than the godet to permit contraction 35 of the thread therebetween and reducing the speed of the godet during the spinning period to effect a decrease in contraction of the thread.

9. In the manufacture of artificial silk, a process for preparing threads, filaments and the like which comprises spinning a cellulosic solution to form a thread, drawing the thread from a coagulating medium and passing the same around at least one godet, leading the thread to a point of collection and collecting the same at a constant rate and during the spinning operation decreasing the speed of the last godet with which the godet contacts to effect a gradual increase in tension whereby objectionable shrinkage characteristics normally existing are avoided.

50 10. In the manufacture of artificial silk, a process for preparing threads, filaments and the

like which comprises spinning a cellulosic solution to form a thread, drawing the thread from a coagulating medium by a driven godet, passing the thread around a second godet having a higher peripheral speed than the first-mentioned godet 5 whereby the thread is stretched, progressively increasing the stretch of the thread between the godets by decreasing the peripheral speed of the first-mentioned godet with which the thread contacts at a given rate while decreasing the peripheral speed of the second godet at a rate lower than the decreasing speed of the first godet during the spinning operation and collecting the thread on a bobbin at a substantially constant rate.

10 11. In the manufacture of artificial silk, a process for preparing threads, filaments and the like which comprises spinning a cellulosic solution to form a thread, drawing the thread from a coagulating medium by a driven godet, passing 20 the thread around a second godet having a higher peripheral speed than the first godet whereby the thread is stretched, progressively increasing the stretch of the thread between the said godets by decreasing the speed of the first-mentioned 25 godet during the spinning operation while maintaining the speed of the second godet constant and collecting the thread on a bobbin rotating at a substantially constant peripheral speed which speed is maintained the same as the peripheral 30 speed of the second godet.

12. The process of producing artificial silk thread and the like of substantially uniform denier and having improved dyeing properties which comprises extruding a cellulosic solution to form 35 a thread, giving the thread a predetermined linear speed at one point in its path of travel between its point of extrusion and a bobbin by passing the same around a godet and directly propelling the same thereby, winding the thread 40 upon the bobbin at a linear speed greater than the linear speed of the thread at the said one point so as to stretch the same, and gradually decreasing the peripheral speed of the godet with the resultant decrease in speed of the thread 45 at said point while operating the bobbin at such peripheral speed that the thread is increasingly elongated as succeeding portions thereof are wound on the bobbin whereby objectionable characteristics resulting from contraction are avoided. 50

GILBERT I. THURMOND.